



The simultaneous vacuum plating of a neodymium cadmium alloy is quite easily accomplished commercially. A typical .0002 to .0005 inch thickness of about 1% neodymium alloy is suitable.

The nonaqueous plating is also a promising solution since it can be accomplished with the plating equipment now being used to apply just the cadmium layer to cadmium plated parts. Such a process is described in Example 2.

**Example 2**

1/4 x 20 4340 notched steel studs, 2 inches long were placed as cathodes in an electrolyte consisting of:

34 gms. (.1M) of  $\text{Nd}_2\text{O}_3$ , and  
180 gms. (3.0M) of  $\text{CO}(\text{NH}_2)_2$  urea

at a temperature of 245° F. Carbon anodes were used and the plating proceeded as follows:

| Time, minutes | Current density, amps/sq. ft. | Voltage, v. | Nd deposit thickness, inch |
|---------------|-------------------------------|-------------|----------------------------|
| 5-----        | 90                            | 5           | Flash                      |
| 15-----       | 190                           | 8           | $5 \times 10^{-6}$         |

Other studs were placed as cathodes in an electrolyte consisting of:

20 gms. (.1M) of  $\text{NdF}_3$ , and  
180 gms. (3.0M) of  $\text{CO}(\text{NH}_2)_2$  urea

at a temperature of 255° F. Carbon anodes were again used and the plating proceeded as follows:

Time, min. 5  
Voltage 4  
Nd Deposit Thickness flash

Still other studs were placed as the cathodes in an electrolyte consisting of:

24.6 gms. (.1M) of  $\text{CeCl}_3$ , and  
220 gms. (3.5M) of  $\text{CO}(\text{NH}_2)_2$  urea

at a temperature of 250° F. Carbon anodes were used and the plating proceeded as follows:

Time 5 min  
Current Density 180 Amps/sq.ft.  
Voltage 17  
Ce Deposit Thickness  $1 \times 10^{-4}$  inch

After rare earth plating, the studs were cadmium plated by placing them as cathodes in an electrolyte made from:

17 gms. (.1M) of  $\text{CdSO}_4 \cdot 8\text{H}_2\text{O}$ , and  
180 gms. (3.0M) of  $\text{CO}(\text{NH}_2)_2$  urea

at a temperature of 250° F. Carbon anodes were used and the plating proceeded as follows:

| Time, minutes | Current density, amps/sq. ft. | Voltage, v. | Cd deposit thickness, inch |
|---------------|-------------------------------|-------------|----------------------------|
| 10-----       | <9                            | 2.5         | $5 \times 10^{-5}$         |
| 5-----        | 9                             | 3.5         | $1.5 \times 10^{-4}$       |

In all cases, there was no discernible difference in appearance between the rare earth-cadmium plated studs and control studs cadmium plated in a conventional aqueous cadmium plating process.

Two studs having a  $5 \times 10^{-5}$  inch Nd plate and a  $1.5 \times 10^{-4}$  Cd plate and two studs having a  $1.5 \times 10^{-4}$  inch Cd plate conventionally applied were placed in a sustained load test with the load at 90% of ultimate. None of the studs were baked. The conventionally plated Cd specimens broke at 12 and 16 hours showing diffusion of hydrogen to high stress areas therein to cause the failures. The Nd-Cd plated specimens withstood the sustained load

without any measurable harm for 266 hours at which time the test was arbitrarily stopped. The above testing proved that nonaqueous rare earth-Cd plating processes are as effective as the vapor deposition in the reduction of hydrogen embrittlement.

Although urea was used as the solvent in the nonaqueous plating process, many other nonaqueous polar solvents can be used including formamide; N,N-dimethylformamide; acetamide; N,N-dimethylacetamide; acetonitrile; dimethylsulfoxide; and dimethylsulfone.

Thus there has been shown and described a novel method for preventing hydrogen embrittlement which fulfills all of the objects and advantages sought therefor. Many changes, alterations, modifications and other uses and applications of the present invention will become apparent to those skilled in the art after considering this specification. All such changes, modifications, variations, and other uses and applications which do not depart from the spirit and scope of the present invention are deemed to be covered by the invention which is limited only by the claims which follow.

What is claimed is:

1. A method of reducing hydrogen embrittlement of items to be protected from corrosion by sacrificial coatings whose cathodic corrosion protection reaction produces free hydrogen, said method comprises applying at least one rare earth metal on the surface of the item either before or during application of said sacrificial coating, said rare earth metal acting as a hydrogen getter to reduce the free hydrogen available to embrittle the corrosion protected item.

2. The method described in Claim 1 wherein a layer of rare earth metal is applied to the surface of the item in an electrochemical plating process using a nonaqueous solvent and at least one rare earth salt as electrolyte.

3. The method defined in Claim 2 wherein said item is thereafter coated with said sacrificial coating in an electrochemical plating process using a nonaqueous solvent as the major constituent of the electrolyte.

4. The method defined in Claim 2 wherein said nonaqueous solvent is chosen from a group consisting of urea, formamide, N,N-dimethylformamide, acetamide, N,N-dimethylacetamide, acetonitrile, dimethylsulfoxide, and dimethylsulfone.

5. The method described in Claim 1 wherein said rare earth metal is vacuum deposited on the surface of the item.

6. The method described in claim 5 wherein a protective layer of metal is deposited over said rare earth metal after which said item is coated with said sacrificial coating.

7. The method described in Claim 1 wherein said rare earth metal is chosen from the group consisting of cerium, neodymium, praseodymium and yttrium.

8. The method defined in Claim 1 wherein said sacrificial coating is a cadmium plate.

9. The method defined in Claim 1 wherein a rare earth metal—sacrificial coating alloy is vacuum deposited on said item's surface.

10. The method of reducing hydrogen embrittlement of a hydrogen sensitive item, said method comprising coating at least one rare earth metal chosen from the group consisting of cerium and neodymium on the surface of the item and applying a protective coating thereover, said rare earth metal acting as a hydrogen getter by forming rare earth hydrides thereby reducing the amount of free hydrogen available to embrittle the hydrogen sensitive item.

11. The method described in Claim 10 wherein said rare earth metal is vacuum deposited on the surface of the item.

12. The method described in Claim 10 wherein a layer of rare earth metal is applied to the surface of the item in an electrochemical plating process using a nonaqueous solvent and at least one rare earth salt as electrolyte.

13. The method defined in Claim 12 wherein said item is thereafter coated with a layer of metal in an electrochemical plating process using an nonaqueous solvent as the major constituent of the electrolyte.

14. The method defined in Claim 12 wherein said nonaqueous solvent is chosen from a group consisting of urea, formamide, N,N-dimethylformamide, acetamide, N,N-dimethylacetamide, acetonitrile, dimethylsulfoxide, and dimethylsulfone.

15. A method of reducing hydrogen embrittlement of items protected from corrosion by sacrificial coatings whose cathodic corrosion protection reaction produces free hydrogen, said method comprises diffusing at least one rare earth metal into the surface of the item and coating said item with said sacrificial coating. 15

## References Cited

## UNITED STATES PATENTS

|             |        |                |          |
|-------------|--------|----------------|----------|
| 2,400,255   | 5/1946 | Pfeil          | 204—56 R |
| 3,732,076   | 5/1973 | Toy et al.     | 23—232 R |
| 5 3,489,538 | 1/1970 | Cook           | 204—39   |
| 3,524,800   | 8/1970 | Morrice et al. | 75—152   |
| 3,049,797   | 8/1962 | Drummond       | 75—152   |

10 JOHN H. MACK, Primary Examiner  
R. L. ANDREWS, Assistant Examiner

U.S. Cl. X.R.

117—71 M, 107; 204—59